

# UNITED STATES PATENT OFFICE.

JAMES EDGAR BLACK AND MICHAEL A. POPKESS, OF KANSAS CITY, MISSOURI,  
ASSIGNORS TO BITUMINIZED ROAD COMPANY, OF KANSAS CITY, MISSOURI, A  
CORPORATION OF ARIZONA.

## PROCESS OF MAKING PAVING COMPOSITIONS AND PRODUCTS THEREOF.

1,320,672.

Specification of Letters Patent.

Patented Nov. 4, 1919.

No Drawing. Application filed April 16, 1917, Serial No. 162,509. Renewed September 16, 1919. Serial No. 324,213.

*To all whom it may concern:*

Be it known that we, JAMES EDGAR BLACK and MICHAEL A. POPKESS, citizens of the United States, and residents of Kansas City, 5 in the county of Jackson and State of Missouri, have invented certain new and useful improvements in Processes of Making Paving Compositions and Products Thereof, of which the following is a specification.

10 This invention relates to processes of making paving compositions and products thereof; and it comprises a method wherein powdered limestone, shells, marl, and other calcareous materials, that is, materials consisting of or comprising calcium carbonate, are impregnated with a binder which may be, and advantageously is, an asphalt which is solid or semisolid at ordinary temperatures, or may be an asphaltic composition liquid 15 at ordinary temperatures, such impregnation being with the aid of vacuum and heat, impregnation being usually aided by pressure; and it further comprises as a new paving material a pulverulent relatively coarse 20 grained limestone or the like having the grains thereof thoroughly impregnated with bitumen, such bitumen filling all the natural pores with substantial completeness; all as more fully hereinafter set forth and as 25 claimed.

The oldest type of asphalt pavement was made with certain natural rocky or stony materials found in Europe and used originally in paving Paris. These natural materials consisted of particles of limestone and bitumen, the particles of the mineral matter being of extreme fineness and thoroughly distributed through the bitumen. In material of the best quality, the proportion 30 of bitumen and of limestone and their mutual relation were such that the material could be placed on a roadway, and tamped, stamped, rammed or rolled into the desired contour of the roadway. This material 35 made an excellent pavement of long-lived and permanent character and one which could be readily repaired or patched with the same material. It did not exude or soften under the summer sun. Its only disadvantages were that the pavement was very 40 hard and unyielding and was apt to be too smooth, particularly in winter and rainy weather. This was for the reason that even

in the best samples there was not quite enough asphalt or bitumen. For a pavement 55 of this character there should be about 13 per cent. to 17 per cent. of asphalt while the average in this natural material rarely reaches 11 per cent. Much of it goes as low as 5 per cent. The natural rock was uneven 60 in character, some portions containing more bitumen and some less; and mixtures were, similarly, uneven. And the average content of asphalt was too little. In making the pavements the rocky material was heated, 65 crushed and ground and thoroughly mixed in order to obtain an average material; but, as stated, the average material, even when 70 of the best character, contained too little bitumen. Additions of asphalt from other sources were tried but did not give satisfactory results for the reason that the foreign asphalt simply diluted the mixture and did not assume the same relation to the 75 mineral matter as that of the original bitumen. However, as stated, these Paris pavements were excellent pavements; they were the best known at their date and have rarely been equaled or surpassed since.

Various attempts have been made to duplicate this natural material but they have 80 been uniformly unsuccessful for various reasons; and modern asphalt pavements in this country where this natural material is not available, are universally of entirely different 85 types. They are built up structures containing aggregates of coarse mineral matter (sand with crushed rock or gravel) in interlocking engagement with the various portions of aggregate cemented by asphalt layers and with the voids filled with asphalt. 90

We have found that the lack of success in the various attempts at duplicating this natural paving material have been due to the fact that impregnation of the particles of 95 limestone could not be made uniform. Any mechanically crushed limestone or like material is composed of grains of no great mechanical strength; the grains are porous and are relatively friable, crushing with comparative readiness. The pores are air-bound. In making a mixture of crushed limestone with asphalt, it is difficult to remove this air and cause the bitumen to enter the pores. But if the pores are not entered by the asphalt and if the amount of asphalt chosen 100

relative to the total amount of limestone is such as will give a hard, resistant pavement, that is the amount which will be, so to speak, taken up by the powder then in use when the 5 particles of limestone crush further there is a production of unimpregnated or uncoated grinding surfaces. The net result is that unless the pavement is made with enough asphalt to provide for subsequent impregnation of the limestone particles as they are 10 broken down under traffic, (in which case the pavement is soft and yielding because of this excess temporarily present), the whole pavement will disintegrate and form 15 dusty or powdery material.

We have found that all these disadvantages may be obviated and a material produced which, although like the natural European material in that it consists mainly of 20 asphalt and calcareous material and possesses the stated advantages, is much more uniform in character and has the said advantage in a much higher degree. And it has certain new advantages of its own. By this 25 invention, it is possible to produce material of any desired relative ratio between calcareous material and bitumen; so that thereby a material may be produced having the optimum ratio of asphalt instead 30 of ratio limited by the amount naturally present as in the case of native materials. In so doing, as we have found, it is only necessary to rely upon the simple expedient of performing the incorporation of 35 asphalt and limestone dust under a vacuum. Operating under a vacuum, the air in the pores of the granules or grains is removed and the asphalt takes its place. Instead of 40 the pores being airbound during the mixing operation, and not being impregnated with bitumen, under the influence of the vacuum the air leaves and the bitumen takes its place. The operation should be conducted with the materials as hot as practicable to 45 give a maximum of liquidity and penetration. Since the operation is under heat and vacuum, the asphalt should be as free as possible of oils volatilizing under the circumstances. For the sake of securing liquidity, 50 we may mix the asphalt with more or less of an oil not volatilizing much at the temperature employed, perform my incorporation under vacuum and thereafter raise the whole mixture to a higher temperature, while still 55 maintaining the vacuum, in order to remove these oils. Or we may indeed use some fluxing oil which is not volatile at all; or at least not to any substantial extent. We may use any solid or semisolid asphalt, that is 60 any asphalt which is solid or semisolid under atmospheric conditions, though we find it often advantageous in many respects to use asphalts which are normally liquid at atmospheric temperatures. Since in the ultimate composition the amount of asphalt is

always merely that which will suffice to impregnate without giving any free liquid layers of substantial thickness, the liquid asphalts are here applicable as well as the solid varieties.

Under the present invention it is not necessary to grind the limestone to extreme fineness; there is not need of striving to secure the extremely great subdivision of the calcium carbonate particles that exist in 75 the stated European materials. It is sufficient to granulate it. Whatever the granule size, however, the material should be fairly uniform. The size of grain which is most 80 advantageous will depend to some extent upon the porosity of the limestone. With a soft highly porous material such as a shell marl or as a chalky limestone, rather coarse grains may be used, since the texture is open enough to permit intercommunication of the 85 pores and removal of air throughout the granules with simultaneous penetration of the asphalt throughout. Something of course also depends upon the coarseness or fineness of pore. As a general rule, the 90 harder the limestone, the finer we grind it; but in all cases it is, as compared with the mineral constituents existing in the natural asphalt rock, a relatively coarse material. A good material may be made even with the 95 very hard limestones by grinding to less than 100 mesh, while with some softer limestones, a granule size of less than 20 mesh may be sufficient.

Any convenient type of mixing apparatus 100 with means for incorporation under vacuum and heat may be used. With the small proportions of asphalt employed, the mixture is rather stiff, even when quite hot and it is desirable that powerful disintegrating and 105 stirring means be used. Ordinarily, we work at about 180-212° F., although we may use higher or lower temperatures, this depending largely upon the particular asphalt used. A proportion of 11 per cent. to 19 110 per cent. asphalt in the finished product is desirable. The materials may be moist during incorporation with some advantage but the presence of the water vapor, unless work is at a low temperature, is inconvenient in 115 maintaining the vacuum.

In a typical embodiment of our invention we grind a limestone of ordinary hardness to a fineness of less than 50 mesh; place this material in a rotatable drum provided 120 with external heating means, create a vacuum of 15 to 25 inches and introduce a suitable amount of normally liquid asphalt, or asphalt that has been liquefied by heating. Steam is then introduced which furnishes 125 pressure to cause impregnation of the pores of the limestone by the asphalt and also serves to retain the asphalt in a liquid condition. The proportion of this asphalt may be 11 to 19 per cent. of the final product. 130

Heating and mixing are continued until the air is sufficiently removed from the pores and the liquid asphalt has disappeared and the impregnation of the particles is complete. With the liquid asphalt the temperature may be around 200° F. Heat in using a liquid asphalt is only desirable as shortening the period of treatment. With asphalts which are solid or semisolid at ordinary temperatures, heat is necessary to produce liquidity, either before or during the mixing. At the end of the incorporation the drum will contain a more or less pulverulent black mass of impregnated limestone grains. This material may be kept and stored indefinitely. In use we heat it somewhat and deposit it on the roadway; thereafter rolling it or tamping it in place. We may press it into blocks and use these. While the material is substantially dry in the sense that it will not give up any substantial amount of asphalt to other materials, yet there is enough film coating on the faces of the grains to make them adhere when they are pressed together. The pavement made by the material is permanent, hard, dense, malleable and resistant to all the stresses and strains of traffic, not disintegrating, softening, rutting or wavering. But it is malleable enough to make repair easy. Under pressure, it can be given any contour or shape desirable.

What we claim is:—

1. The process of making a paving material which comprises disintegrating a natural calcareous material and mixing the resultant material with a binder having adhesive and waterproof qualities under a substantial vacuum, the quantity of binder used being just sufficient to fill the pores of the calcareous material.

2. The process of making a paving material which comprises crushing a natural calcareous material and mixing the resultant material with asphalt under vacuum and

heat, the quantity of binder used being just sufficient to fill the pores of the calcareous material.

3. The process of making a paving material which comprises disintegrating a natural calcareous material and mixing the resultant material with a binder having adhesive and waterproof qualities under vacuum, the quantity of binder used being just sufficient to fill the pores of the calcareous material.

4. The process of making a paving material which comprises pulverizing a natural calcareous material and mixing the resultant material with from 11 to 19 per cent. of normally liquid asphalt under vacuum and heat.

5. The process of making a paving material which comprises comminuting limestone and mixing the resultant material under vacuum with the proper proportion of asphalt to make it non-flowing, malleable and traffic supporting.

6. The process of making a paving material which comprises disintegrating limestone and mixing the resultant material under vacuum and heat with the proper proportion of asphalt to make it non-flowing, malleable and traffic supporting.

7. The process of making a paving material which comprises disintegrating limestone and mixing the resultant material with from 11 to 19 per cent. of normally liquid asphalt under vacuum.

8. The process of making a paving material which comprises disintegrating limestone and mixing the resultant powder with the right proportion of normally liquid asphalt to make it dense, malleable, waterproof, and non-flowing, mixing being under vacuum and heat.

In testimony whereof we affix our signatures hereto.

JAMES EDGAR BLACK.  
MICHAEL A. POPKESS.